

Patented June 15, 1943

2,321,816

# UNITED STATES PATENT OFFICE

2,321,816

## PROCESS OF PRODUCING FAST DYEINGS ON FIBROUS MATERIALS

Richard Huss, Frankfort-on-the-Main, Germany,  
assignor to General Aniline & Film Corporation,  
New York, N. Y., a corporation of Delaware

No Drawing. Application February 7, 1941, Serial  
No. 377,848. In Germany February 22, 1940

11 Claims. (Cl. 8—46)

The present invention relates to a process of producing fast dyeings and to the dyed fiber obtained thereby.

I have found that valuable dyeings of good properties of fastness may be obtained on animal fibers and natural or artificial cellulose fibers as well as on mixtures of animal fibers with cellulose fibers, furthermore on structures from synthetic polyamide compounds of high molecular weight by applying to the fiber secondary disazo-dyestuffs of the following composition:



wherein A means the radical of a 1-amino-5-hydroxynaphthalene, B the radical of an amine of the benzene or naphthalene series being free from hydroxy groups and coupled in para-position to the amino-group, C means the radical of an amino-hydroxynaphthalene sulfonic acid coupled on the naphthol side, X represents hydrogen or alkyl and Y an acyl or an aryl radical, the dyestuff components being selected in such a manner that the finished dyestuff contains at least two solubilizing groups, and developing the dyeings thus obtained with water-soluble diazo-compounds containing at least one nitro-group, but no sulfonic acid or carboxylic acid group.

The blue to black dyeings thus obtained are distinguished by good properties of fastness, especially by very good fastness to light and to decolorizing. On mixed fabrics from wool and natural or regenerated celluloses there are obtained, after developing, dyeings the various fibers of which are very uniform as regards their shade and intensity of color.

If the dyeings obtainable by the present invention are treated with agents yielding metal either before or after or simultaneously with the development with the water-soluble diazo-compounds containing at least one nitro-group, but no sulfonic acid or carboxylic acid group, dyeings are obtained which possess enhanced properties of fastness, partly a better fastness to wet-processing, partly a better fastness to light. As agents yielding metal there may, for instance, be used salts of aluminium, copper, cobalt, nickel, chromium, manganese and mixtures of these salts.

The following examples serve to illustrate the invention, but they are not intended to limit it thereto.

1. 1 kilo of a mixed fiber consisting of 50 parts of wool and 50 parts of staple fiber from cuprammonium cellulose is treated for one hour at 95° C. in a bath containing in 30 liters of water 40 gams of the azo-dyestuff obtainable by coupling diazotized 1-amino-5-hydroxynaphthalene-7-sulfonic acid in an acid medium with 1-amino-naphthalene-7-sulfonic acid, diazotizing again the monoazo-dyestuff obtained and coupling this di-

- 5 azo-compound in an alkaline medium with 2-acetylaminio-5-hydroxynaphthalene-7-sulfonic acid,
- 10 grams of the condensation product from 1 mol of octodecyl alcohol and 20 mols of ethylene oxide,
- 100 grams of ammonium sulfate and 600 grams of sodium sulfate.
- 10 The material is then allowed to stand for half an hour at a temperature slowly falling to 80° C. and thereupon it is rinsed. The dyeing is then developed for half an hour in the cold in a solution containing in 30 liters of water:
- 15 30 grams of the diazonium borofluoride from 1-amino-2-methyl-4-nitrobenzene
- 10 grams of the condensation product from 1 mol of octodecyl alcohol and 20 mols of ethylene oxide
- 20 5 grams of glacial acetic acid and 100 grams of sodium acetate . and rinsed again. There is obtained a black dyeing of very good properties of fastness, especially of very good fastness to decolorizing and to light.
- 25 By after-treating the dyeing obtained with potassium bichromate in the heat, somewhat deeper dyeings with enhanced properties of fastness are obtained.
- 30 On wool dyeings of similar properties are obtained. For the production of dyeings on cotton or regenerated cellulose an addition of ammonium sulfate to the dye-bath is not necessary.
- 35 2. 1 kilo of an artificial wool containing beside wool artificial silk staple fiber and cotton is dyed for one hour at 95° C. in a solution containing in 30 liters of water 40 grams of the sodium salt of the azo-dyestuff obtainable by coupling diazotized 1-amino-5-hydroxynaphthalene-7-sulfonic acid with 1-aminonaphthalene-7-sulfonic acid, diazotizing again the monoazodyestuffs obtained and coupling this diazo-compound with 2-acetylaminio-8-hydroxynaphthalene-6-sulfonic acid,
- 40 10 grams of the condensation product from 1 mol of octodecyl alcohol and 20 mols of ethylene oxide
- 45 100 grams of ammonium sulfate and 600 grams of sodium sulfate
- 50 The material is allowed to stand for half an hour while the temperature decreases, rinsed and treated for half an hour in the cold in a bath containing in 30 liters of cold water
- 55 30 grams of the diazonium zinc chloride double salt from 3-nitraniline
- 5 5 grams of glacial acetic acid
- 10 10 grams of the condensation product from 1 mol of octodecyl alcohol and 20 mols of ethylene oxide and
- 60 100 grams of sodium acetate

It is then rinsed cold and hot. A black dyeing of very good properties of fastness is obtained

which may be improved by a treatment at boiling temperature with a solution of 20 grams of sodium bichromate, 10 grams of glacial acetic acid and 10 grams of the condensation product from 1 mol of octodecyl alcohol and 20 mols of ethylene oxide in 30 liters of water.

3. 1 kilo of a mixed fabric consisting of 50 parts of wool and 50 parts of staple fiber from viscose is treated for one hour at 95° C. and thereupon for half an hour at a temperature falling to 80° C. in a bath containing in 30 liters of water 30 grams of the sodium salt of the azo-dyestuff obtainable by coupling diazotized 1-amino-5-hydroxynaphthalene-7-sulfonic acid in an acid medium with 1-amino-2-methoxy-5-methylbenzene, diazotizing again this monoazo-dyestuff and coupling the diazo-compound obtained in an alkaline medium with 1-benzoyl-amino-8-hydroxy-naphthalene-4-sulfonic acid,

10 grams of the condensation product from 1 mol of octodecylalcohol and 20 mols of ethylene oxide

10 grams of glacial acetic acid

500 grams of sodium sulfate and

100 grams of ammonium sulfate

The material is then rinsed, developed for half an hour in a fresh bath with

25 grams of the diazonium borofluoride from 4-nitraniline

10 grams of the condensation product from 1 mol of octodecylalcohol and 20 mols of ethylene oxide and

100 grams of sodium acetate in 30 liters of cold water

treated at 45° C. for 1/4 hour with a solution of 5 grams of the condensation product from 1 mol of octodecylalcohol and 20 mols of ethylene oxide and 80 cc. of an ammonia solution of 25 per cent strength in 30 liters of water, rinsed and dried. A black dyeing of very good fastness to decatizing, to perspiration and to light is obtained. If the mixed fabric contains cotton knops, these are covered.

4. Mixed yarn consisting of 30 parts of staple fiber from viscose and 70 parts of wool is dyed for one hour at 95° C. with 2 per cent of the azo-dyestuff 1-amino-5-hydroxynaphthalene-7-sulfonic acid→1-naphthylamino-7-sulfonic acid→2-(4'-hydroxy-5'-carboxyphenylamino)-5-hydroxynaphthalene-7-sulfonic acid, 0.5 per cent of the condensation product from 1 mol of octodecylalcohol and 20 mols of ethylene oxide,

10 per cent of ammonium sulfate and

50 per cent of sodium sulfate

the proportion of the goods to the liquor being 1:30.

The material is cooled to 80° C., rinsed and developed for half an hour in the cold with

1 per cent of diazotized 1-amino-4-nitrobenzene 0.5 per cent of the condensation product from 1 mol of octodecylalcohol and 20 mols of ethylene oxide and

10 per cent of sodium acetate

slowly heated to 45° C., kept at this temperature for half an hour, rinsed and after-treated for one hour at 85° C. to 90° C. with

3 per cent of chromic chloride and

1 per cent of glacial acetic acid

A blue-black dyeing of very good properties of fastness is obtained. If there is used diazotized

1-amino-2-methyl-4-nitrobenzene instead of diazotized 1-amino-4-nitrobenzene, and aluminum acetate instead of chromic chloride, a blue-black dyeing of similar properties is obtained.

5. Piece goods from fleece wool, shoddy, staple fiber from viscose and cuprammonium silk are dyed on a winch dye beck for about one hour at 95° C. with 4 per cent of the azo-dyestuff 1-amino-5-hydroxynaphthalene-7-sulfonic acid→1-amino-2,5-di-methoxybenzene→2-(4'-aminobenzoylamino)-8-hydroxynaphthalene-6-sulfonic acid,

10 per cent of ammonium sulfate

50 per cent of sodium sulfate and

15 0.5 per cent of the condensation product from 20 mols of ethylene oxide and 1 mol of octodecylalcohol

the proportion of the goods to the liquor being 1:30.

20 The material is cooled to about 80° C. in the course of about half an hour, rinsed and developed for half an hour at ordinary temperature with

25 1 per cent of diazotized 1-amino-4-nitrobenzene in the form of the hydrochloride

0.5 per cent of the condensation product from 20 mols of ethylene oxide and 1 mol of octodecylalcohol

30 10 per cent of sodium acetate and 2 per cent of copper sulfate.

Then it is slowly heated to about 95° C., treated for about 3/4 to one hour at this temperature and rinsed. A black dyeing of very good properties of fastness, especially of very good fastness to light is obtained.

By exchanging the diazo-compound from 1-amino-4-nitrobenzene for the diazo-compound from 1-amino-3-nitrobenzene or 1-amino-2-methyl-4-nitrobenzene, similar black shades are obtained. By using the diazo compound from 1-amino-2-methyl-5-nitrobenzene or 1-amino-2-nitro-4-chlorobenzene blue-black dyeings of very good properties and very good evenness of all fibers are obtained.

45 6. Piece goods from wool and staple fiber from viscose containing effects from acetate artificial silk are dyed for one hour at 95° C. on a winch dye beck with

2 per cent of the azo-dyestuff 1-amino-5-hydroxynaphthalene-7-sulfonic acid→2-amino-4-methylphenoxy acetic acid→2-(4'-hydroxy-3'-carboxyphenylamino)-5-hydroxynaphthalene-7-sulfonic acid

0.5 per cent of the condensation product from 20 mols of ethylene oxide and 1 mol of octodecylalcohol

55 10 per cent of ammonium sulfate and

50 per cent of sodium sulfate

the proportion of the goods to the liquor being 1:30. The whole is then cooled to about 80° C., rinsed and developed for half an hour in the cold with

65 1 per cent of diazotized 1-amino-3-nitro-6-methylbenzene in the form of its hydrochloride 0.5 per cent of the condensation product from 20 mols of ethylene oxide and 1 mol of octodecylalcohol

70 10 per cent of sodium acetate

1 per cent of copper sulfate and

1 per cent of chromic fluoride

75 slowly heated to 45° C., further treated at this

temperature for about one hour and rinsed. A fast vivid navy-blue dyeing containing white effects from acetate silk is obtained. By exchanging the diazotized 1-amino-3-nitro-6-methylbenzene for the same quantity of diazotized 1-amino-3-nitrobenzene, a somewhat more covered shade is obtained.

7. Mixed yarn consisting of 50 parts of wool and 50 parts of staple fiber from viscose is dyed for one hour at 95° C. with

4 per cent of the azo-dyestuff 1-amino-5-hydroxynaphthalene-7-sulfonic acid → 1-amino-naphthalene-7-sulfonic acid → 2-acetylaminio-5-hydroxynaphthalene-7-sulfonic acid

0.5 per cent of the condensation product from 1 mol of octodecylalcohol and 20 mols of ethylene oxide

10 per cent of ammonium sulfate and 50 per cent of sodium sulfate

The material is cooled to 80° C., rinsed and developed, first for half an hour in the cold, then for half an hour at 45° C. with

1 per cent of diazotized 1-amino-4-nitrobenzene

0.5 per cent of the condensation product from 1 mol of octodecylalcohol and 20 mols of ethylene oxide and

10 per cent of sodium acetate

rinsed and treated for one hour at 90° C. with 2.30 vention:

per cent of potassium bichromate and 1 per cent of glacial acetic acid. A reddish black dyeing of good properties of fastness is obtained.

Black dyeings of considerably enhanced fastness to light are obtained on mixtures of staple fiber from viscose and wool by developing a dyeing of 4 per cent of the azo-dyestuff 1-amino-5-hydroxynaphthalene-7-sulfonic acid → 1-amino-2-methoxy-5-methylbenzene → 1-benzoylaminio-8-hydroxynaphthalene-4-sulfonic acid with diazotized 1-amino-2-methyl-4-nitrobenzene and after-treating the dyeing at 70° C. with 2 per cent of copper acetate and 1 per cent of glacial acetic acid.

15 Dyeings of similar fastness to light are obtained by developing a dyeing in the manner indicated in Example 5 of the before-mentioned azo-dyestuff on a mixture of staple fiber from viscose and wool with diazotized 1-amino-2-methyl-5-nitrobenzene,

0.5 per cent of the condensation product from 1 mol of octodecyl alcohol and 20 mols of ethylene oxide

25 10 per cent of sodium acetate

2 per cent of copper sulfate and 2 per cent of chromic fluoride

The following table indicates the shades of a number of other dyeings obtainable by this in-

vention:

|    | Parent dyestuff                                                                                                                                                   | Developed with the diazocompound from— | Shade of the dyeing on wool, cotton and mixed fibers from wool and artificial silk staple fiber |
|----|-------------------------------------------------------------------------------------------------------------------------------------------------------------------|----------------------------------------|-------------------------------------------------------------------------------------------------|
| 1  | 1-amino-5-hydroxynaphthalene-7-sulfonic acid → 1-amino-naphthalene-7-sulfonic acid → 2-(4'-hydroxy-3'-carboxy-phenyl-amino)-5-hydroxynaphthalene-7-sulfonic acid. | 1-amino-2-methyl-4-nitrobenzene.       | Navy-blue.                                                                                      |
| 2  | 1-amino-5-hydroxynaphthalene-7-sulfonic acid → 1-amino-naphthalene-7-sulfonic acid → 6-ureido-1-hydroxynaphthalene-3-sulfonic acid.                               | 1-amino-2-methoxy-4-nitrobenzene.      | Reddish black.                                                                                  |
| 3  | 1-amino-5-hydroxynaphthalene-7-sulfonic acid → 1-amino-naphthalene-7-sulfonic acid → 1-acetylaminio-5-hydroxy-naphthalene-7-sulfonic acid.                        | 1-amino-3-nitrobenzene.                | Do.                                                                                             |
| 4  | 1-amino-5-hydroxynaphthalene-7-sulfonic acid → 1-amino-naphthalene-7-sulfonic acid → 2-(4'-methoxyphenylamino)-8-hydroxynaphthalene-4-sulfonic acid.              | 1-amino-4-nitrobenzene.                | Black.                                                                                          |
| 5  | 1-amino-5-hydroxynaphthalene-7-sulfonic acid → 1-amino-naphthalene-7-sulfonic acid → 1-(2', 4'-dichlorobenzoylaminio)-8-hydroxynaphthalene-4,6-disulfonic acid.   | 1-amino-3-nitrobenzene.                | Blue-black.                                                                                     |
| 6  | 1-amino-5-hydroxynaphthalene-7-sulfonic acid → 1-amino-2-methoxy-5-methylbenzene → 2-(4'-hydroxy-3'-carboxyphenylamino)-8-hydroxynaphthalene-7-sulfonic acid.     | 1-amino-2-methyl-4-nitrobenzene.       | Violet-tinged dark blue.                                                                        |
| 7  | 1-amino-5-hydroxynaphthalene-7-sulfonic acid → 1-amino-2-methoxy-5-methylbenzene → 1-(2', 4'-dichlorobenzoylaminio)-8-hydroxynaphthalene-4,6-disulfonic acid.     | 1-amino-2-methoxy-4-nitrobenzene.      | Reddish, blue-black.                                                                            |
| 8  | 1-amino-5-hydroxynaphthalene-7-sulfonic acid → 1-amino-3-methylbenzene → 1-acetylaminio-5-hydroxynaphthalene-4-sulfonic acid.                                     | 1-amino-3-nitrobenzene.                | Violet-tinged black.                                                                            |
| 9  | 1-amino-5-hydroxynaphthalene-7-sulfonic acid → 1-amino-2-methoxy-5-methylbenzene → 1-benzoylaminio-8-hydroxynaphthalene-4-sulfonic acid.                          | 1-amino-2-nitro-4-methoxybenzene.      | Blue-black.                                                                                     |
| 10 | do                                                                                                                                                                | 1-amino-2-nitro-4-chlorobenzene.       | Do.                                                                                             |
| 11 | do                                                                                                                                                                | 1-amino-2-nitro-4-methylbenzene.       | Do.                                                                                             |
| 12 | do                                                                                                                                                                | 1-amino-2-nitrobenzene.                | Reddish deep black.                                                                             |
| 13 | 1-amino-5-hydroxynaphthalene-7-sulfonic acid → 1-amino-2,5-dimethoxybenzene → 2-acetylaminio-5-hydroxynaphthalene-7-sulfonic acid.                                | 1-amino-4-nitrobenzene.                | Bluish black.                                                                                   |
| 14 | 1-amino-5-hydroxynaphthalene-7-sulfonic acid → 1-amino-2,5-dimethoxybenzene → 2-benzoylaminio-8-hydroxynaphthalene-6-sulfonic acid.                               | 1-amino-2-nitro-4-chlorobenzene.       | Reddish dark blue.                                                                              |
| 15 | do                                                                                                                                                                | 1-amino-3-nitro-6-methylbenzene.       | Blue-black.                                                                                     |
| 16 | 1-amino-5-hydroxynaphthalene-7-sulfonic acid → 1-amino-naphthalene-7-sulfonic acid → 1-butyrylaminio-8-hydroxynaphthalene-4-sulfonic acid.                        | do                                     | Do.                                                                                             |
| 17 | 1-amino-5-hydroxynaphthalene-7-sulfonic acid → 1-amino-2-ethoxy-naphthalene-6-sulfonic acid → 2-acetylaminio-8-hydroxynaphthalene-6-sulfonic acid.                | 1-amino-4-nitrobenzene.                | Black.                                                                                          |
| 18 | 1-amino-5-hydroxynaphthalene-7-sulfonic acid → 1-amino-2-ethoxy-naphthalene-6-sulfonic acid → 2-acetylaminio-5-hydroxynaphthalene-7-sulfonic acid.                | do                                     | Do.                                                                                             |
| 19 | 1-amino-5-hydroxynaphthalene-7-sulfonic acid → 1-amino-2,5-dimethoxybenzene → 2-(4'-aminobenzoylaminio)-8-hydroxynaphthalene-6-sulfonic acid.                     | 1-amino-3-nitrobenzene.                | Do.                                                                                             |
| 20 | 1-amino-5-hydroxynaphthalene-7-sulfonic acid → 2-amino-4-methylphenoxy acetic acid → 2-(4'-hydroxy-3'-carboxyphenylamino)-5-hydroxynaphthalene-7-sulfonic acid.   | 1-amino-3-nitro-6-methylbenzene.       | Reddish navy-blue.                                                                              |
| 21 | 1-amino-5-hydroxynaphthalene-7-sulfonic acid → 1-amino-6-sulfo-2-naphthoxy acetic acid → 2-phenylaminio-5-hydroxynaphthalene-7-sulfonic acid.                     | 1-amino-2-methyl-4-nitrobenzene.       | Dark blue.                                                                                      |

|    | Parent dyestuff                                                                                                                                                 | Developed with the diazocompound from—                                              | Simultaneously treated with                                     | Shade of the dyeing on wool, cotton and mixed fibers from wool and artificial silk staple fiber |
|----|-----------------------------------------------------------------------------------------------------------------------------------------------------------------|-------------------------------------------------------------------------------------|-----------------------------------------------------------------|-------------------------------------------------------------------------------------------------|
| 22 | 1-amino-5-hydroxy-naphthalene-7-sulfonic acid → 2-phenylamino-8-hydroxynaphthalene-6-sulfonic acid.                                                             | 1-amino-2,5-dimethoxy-benzene → 2-phenylamino-8-hydroxynaphthalene-6-sulfonic acid. | 1-amino-2-methyl-4-nitrobenzene.                                | Copper sulfate → Black.                                                                         |
| 23 | 1-amino-5-hydroxy-naphthalene-7-sulfonic acid → 1-amino-2,5-dimethoxy-benzene → 2-phenyl-amino-8-hydroxynaphthalene-6-sulfonic acid.                            | 1-amino-3-nitrobenzene.                                                             | do.                                                             | Do.                                                                                             |
| 24 | Do.                                                                                                                                                             | 1-amino-2-methoxy-4-nitrobenzene.                                                   | do.                                                             | Do.                                                                                             |
| 25 | 1-amino-5-hydroxy-naphthalene-7-sulfonic acid → 1-amino-2,5-dimethoxy-benzene → 2-acetylamino-5-hydroxynaphthalene-7-sulfonic acid.                             | 1-amino-4-nitrobenzene.                                                             | do.                                                             | Reddish black.                                                                                  |
| 26 | Do.                                                                                                                                                             | do.                                                                                 | Mixture of copper sulfate and chromic fluoride. Copper sulfate. | Reddish black.                                                                                  |
| 27 | 1-amino-5-hydroxy-naphthalene-7-sulfonic acid → 1-amino-2,5-dimethoxy-benzene → 2-benzoyl-amino-8-hydroxynaphthalene-6-sulfonic acid.                           | do.                                                                                 | do.                                                             | Black.                                                                                          |
| 28 | 1-amino-5-hydroxy-naphthalene-7-sulfonic acid → 1-amino-2,5-dimethoxy-benzene → 2-butyl-amino-8-hydroxynaphthalene-6-sulfonic acid.                             | 1-amino-2-methyl-5-nitrobenzene.                                                    | do.                                                             | Reddish black.                                                                                  |
| 29 | 1-amino-5-hydroxy-naphthalene-7-sulfonic acid → 1-amino-2-ethoxy naphthalene-6-sulfonic acid → 2-acetyl-amino-8-hydroxy-naphthalene-6-sulfonic acid.            | do.                                                                                 | do.                                                             | Black.                                                                                          |
| 30 | 1-amino-5-hydroxy-naphthalene-7-sulfonic acid → 1-amino-2-sulfo-2-naphthoxy acetic acid → 2-phenyl-amino-5-hydroxynaphthalene-7-sulfonic acid.                  | 1-amino-2-methyl-4-nitrobenzene.                                                    | do.                                                             | Dark blue.                                                                                      |
| 31 | 1-amino-5-hydroxynaphthalene-7-sulfonic acid → 1-aminonaphthalene-7-sulfonic acid → 1-acetyl-amino-5-hydroxynaphthalene-7-sulfonic acid.                        | do.                                                                                 | After treated with Potassium bichromate.                        | Reddish black.                                                                                  |
| 32 | 1-amino-5-hydroxy-naphthalene-7-sulfonic acid → 1-aminonaphthalene-7-sulfonic acid → 1-(4'-methoxyphenylamino)-8-hydroxynaphthalene-6-sulfonic acid.            | 1-amino-2-methoxy-4-nitrobenzene.                                                   | do.                                                             | Black.                                                                                          |
| 33 | 1-amino-5-hydroxy-naphthalene-7-sulfonic acid → 1-amino-2-methoxy-5-methylbenzene → 2-(4'-hydroxy-3'-carboxy-phenylamino)-5-hydroxynaphthalene-7-sulfonic acid. | 1-amino-3-nitrobenzene.                                                             | do.                                                             | Violet-tinged dark blue.                                                                        |

I claim:

1. A process of producing fast dyeings on fibrous material of the group consisting of animal fibers, natural and artificial cellulose fibers and mixtures of animal fibers with cellulose fibers by applying to the fiber secondary disazo-dyestuffs of the following composition:



wherein A means the radical of a 1-amino-5-hydroxynaphthalene, B the radical of an amine selected from the group consisting of the benzene and naphthalene series being free from hydroxy groups and coupled in para-position to the amino-group, C means the radical of an amino-hydroxynaphthalene sulfonic acid coupled on the naphthol side, X represents a member of the group consisting of hydrogen and alkyl and Y a member of the group consisting of an acyl and aryl radical, the dyestuff components being selected in such a manner that the finished dyestuff contains at least two solubilizing groups, and developing the dyeings thus obtained with water-soluble diazo-compounds of the benzene series containing a nuclear nitro group, said diazo compounds being free from sulfonic acid and carboxylic acid groups.

2. A process of producing fast dyeings on fibrous material of the group consisting of animal fibers, natural and artificial cellulose fibers and mixtures of animal fibers with cellulose fibers by applying to the fiber secondary disazo-dyestuffs of the following composition:



wherein A means the radical of a 1-amino-5-hydroxynaphthalene, B the radical of an amine selected from the group consisting of the benzene

and naphthalene series being free from hydroxy groups and coupled in para-position to the amino-group, C means the radical of an amino-hydroxynaphthalene sulfonic acid coupled on the naphthol side, X represents a member of the group consisting of hydrogen and alkyl and Y a member of the group consisting of an acyl and aryl radical, the dyestuff components being selected in such a manner that the finished dyestuff contains at least two solubilizing groups, developing the dyeings thus obtained with water-soluble diazo-compounds of the benzene series

40 containing a nuclear nitro-group, said diazo compounds being free from sulfonic acid and carboxylic acid groups and treating them with agents yielding metal.

3. A process of producing fast blue-black dyeings on fibrous material of the group consisting of animal fibers, natural and artificial cellulose fibers and mixtures of animal fibers with cellulose fibers by applying to the fiber the secondary disazo-dyestuff 1-amino-5-hydroxynaphthalene-7-sulfonic acid → 1-amino-2-methoxy-5-methylbenzene → 1-benzoyl-amino-8-hydroxynaphthalene-4-sulfonic acid and developing the dyeing thus obtained with the diazo-compound from a nitraniline.

4. A process of producing fast blue-black dyeings on fibrous material of the group consisting of animal fibers, natural and artificial cellulose fibers and mixtures of animal fibers with cellulose fibers by applying to the fiber the secondary disazo-dyestuff 1-amino-5-hydroxynaphthalene-7-sulfonic acid → 1-amino-2-methoxy-5-methylbenzene → 1-benzoyl-amino-8-hydroxynaphthalene-4-sulfonic acid and developing the dyeing thus obtained with the diazo-compound from 70 1-amino-4-nitrobenzene.

5. A process of producing fast blue-black dyeings on fibrous material of the group consisting of animal fibers, natural and artificial cellulose fibers and mixtures of animal fibers with cellulose fibers by applying to the fiber the secondary

disazo-dyestuff 1-amino-5-hydroxynaphthalene-7-sulfonic acid → 1-amino-2-methoxy-5-methylbenzene → 1-benzoylamino-8-hydroxynaphthalene-4-sulfonic acid, developing the dyeing thus obtained with the diazo-compound from 1-amino-4-nitrobenzene and treating it with an agent yielding metal.

6. A process of producing fast black dyeings on fibrous material of the group consisting of animal fibers, natural and artificial cellulose fibers and mixtures of animal fibers with cellulose fibers by applying to the fiber the secondary disazo-dyestuff 1-amino-5-hydroxynaphthalene-7-sulfonic acid → 1-amino-2,5-dimethoxybenzene → 2-(4'-aminobenzoylamino)-8-hydroxynaphthalene-6-sulfonic acid, and developing the dyeing thus obtained with the diazo-compound from a nitraniline.

7. A process of producing fast black dyeings on fibrous material of the group consisting of animal fibers, natural and artificial cellulose fibers and mixtures of animal fibers with cellulose fibers by applying to the fiber the secondary disazo-dyestuff 1-amino-5-hydroxynaphthalene-7-sulfonic acid → 1-amino-2,5-dimethoxybenzene → 2-(4'-aminobenzoylamino)-8-hydroxynaphthalene-6-sulfonic acid and developing the dyeing thus obtained with the diazo-compound from 1-amino-4-nitrobenzene.

8. A process of producing fast black dyeings on fibrous material of the group consisting of animal fibers, natural and artificial cellulose fibers and mixtures of animal fibers with cellulose fibers by applying to the fiber the secondary disazo-dyestuff 1-amino-5-hydroxynaphthalene-7-sulfonic acid → 1-amino-2,5-dimethoxybenzene → 2-(4'-aminobenzoylamino)-8-hydroxynaphthalene-6-sulfonic acid, developing the dyeing thus obtained with the diazo-compound from

1-amino-4-nitrobenzene and treating it with an agent yielding metal.

9. A process of producing vivid navy-blue dyeings on fibrous material of the group consisting of animal fibers, natural and artificial cellulose fibers and mixtures of animal fibers with cellulose fibers by applying to the fiber the secondary disazo-dyestuff 1-amino-5-hydroxynaphthalene-7-sulfonic acid → 2-amino-4-methylphenoxy acetic acid → 2-(4'-hydroxy-3'-carboxyphenylamino)-5-hydroxynaphthalene-7-sulfonic acid and developing the dyeing thus obtained with the diazo-compound from a nitraniline.

10. A process of producing vivid navy-blue dyeings on fibrous material of the group consisting of animal fibers, natural and artificial cellulose fibers and mixtures of animal fibers with cellulose fibers by applying to the fiber the secondary disazo-dyestuff 1-amino-5-hydroxynaphthalene-7-sulfonic acid → 2-amino-4-methylphenoxy acetic acid → 2-(4'-hydroxy-3'-carboxyphenylamino)-5-hydroxynaphthalene-7-sulfonic acid, and developing the dyeing thus obtained with the diazo-compound from 1-amino-3-nitro-6-methylbenzene.

11. A process of producing vivid navy-blue dyeings on fibrous material of the group consisting of animal fibers, natural and artificial cellulose fibers and mixtures of animal fibers with cellulose fibers by applying to the fiber the secondary disazo-dyestuff 1-amino-5-hydroxynaphthalene-7-sulfonic acid → 2-amino-4-methylphenoxy acetic acid → 2-(4'-hydroxy-3'-carboxyphenylamino)-5-hydroxynaphthalene-7-sulfonic acid, developing the dyeing thus obtained with the diazo-compound from 1-amino-3-nitro-6-methylbenzene and treating it with an agent yielding metal.

RICHARD HUSS.